

(No Model.)

P. LANGE.

CORE FOR ELECTRO MAGNETS AND METHOD OF FORMING THE SAME.

No. 366,408.

Patented July 12, 1887.



Fig. 1.



Fig. 2.



Fig. 3.

Witnesses

Geo. W. Breck  
Carrie E. Ashley

By his Attorneys

Inventor  
Philip Lange  
Robert Edgecomb

# UNITED STATES PATENT OFFICE.

PHILIP LANGE, OF PITTSBURG, PENNSYLVANIA, ASSIGNOR TO GEORGE WESTINGHOUSE, JR., OF SAME PLACE.

## CORE FOR ELECTRO-MAGNETS AND METHOD OF FORMING THE SAME.

SPECIFICATION forming part of Letters Patent No. 366,408, dated July 12, 1887.

Application filed December 2, 1886. Serial No. 230,444. (No model.)

*To all whom it may concern:*

Be it known that I, PHILIP LANGE, a subject of the Emperor of Germany, residing in Pittsburg, in the county of Allegheny and State of Pennsylvania, have invented certain new and useful Improvements in Cores for Electrical Instruments and Method of Forming the Same, of which the following is a specification.

10 The invention relates to the construction of cores and armatures for electro-magnetic apparatus—such, for instance, as induction-coils, electrical converters, and electro-magnets in general.

15 The object of the invention is to provide a core or armature susceptible of rapid changes in its magnetic condition, and which will not become overheated by a rapid and continuous magnetic charge and discharge.

20 It has heretofore been proposed to form the cores of electro-magnets from compact bundles of soft-iron wires. For the purpose of the present invention it is desirable that such wires should be to a greater or less extent 25 magnetically insulated from each other, and also that the wires should lie as nearly parallel as possible.

25 The invention therefore consists, in general terms, in constructing cores and armatures in the following manner: A cylinder of suitable non-magnetic and non-conducting material—such, for instance, as paper—is wound continuously from end to end with a single helical layer of soft-iron wire of the required size. The cylinder is preferably first covered

35 by a coating of shellac, varnish, or similar material, and this serves, when dry and hardened, to hold the wire in position. The cylinder thus formed is then cut apart or slit in the direction of its length, and the sheet thus formed is wound or wrapped into a convolute, the wires lying parallel to its axis, the sheet being bent so that the non-conducting material will come inside. The bending of the paper in this manner will necessarily separate the wires from each other a greater or less distance, and these spaces may with advantage be

filled with an additional coating of shellac. This procedure secures a thorough magnetic separation and insulation of the wires.

35 In the accompanying drawings, Figure 1 illustrates the method of forming the sheets. Fig. 2 illustrates the sheet after it has been cut apart, and Fig. 3 illustrates a complete core.

40 Referring to the figures, A represents a hollow cylinder, of paper or other similar flexible non-magnetic material. It is preferably carried by a cylindrical block, B. This may be made compressible like a chuck, or it may be grooved lengthwise to facilitate removing or cutting the sheet. The outer surface of the paper is first coated with any suitable varnish, shellac, or other suitable material, and the wire D is evenly wound upon it. The 45 wire may be itself first covered with a coating of shellac or varnish. The wire is of soft iron, and preferably of very small size. After the varnish or other coating has dried, the sheet is cut apart—for example, along the line 50 a a—and flattened out, as shown in Fig. 2. The sheet or portions thereof, cut to the proper length and breadth, is then rolled up, in the manner shown in Fig. 3. This separates the wires slightly from each other, and the spaces 55 thus formed are preferably filled by the application of shellac or other equivalent material. Usually it is found desirable to coat the sheet with a coating of adhesive material, for which shellac or varnish answers the purpose 60 well, and this serves to bind the convolutions together.

65 A core of this character may be made of any desired form for any of the usual purposes of electro-magnetic apparatus. The 70 sheet may be wrapped on a non-conducting cylinder—such as glass, for instance—when it is desired to produce a hollow core.

75 I claim as my invention—

80 1. A core for electro-magnetic apparatus, consisting of a convolute of non-conducting material covered by wires of soft iron.

85 2. A core for electro-magnetic apparatus, consisting of a sheet of paper, or other non-

magnetic material, covered with soft-iron wires and wrapped upon itself, substantially as described.

3. As an article of manufacture, a sheet of non-magnetic non-conducting material covered upon one side by wires of soft iron, substantially as described.

4. The hereinbefore-described method of forming cores for electro-magnets, which consists in winding wire upon a non-conducting

sheet, cutting the wires across their lengths, and wrapping the sheet upon itself, substantially as set forth.

In testimony whereof I have hereunto subscribed my name this 29th day of October, A. D. 1886.

PHILIP LANGE.

Witnesses:

CHARLES A. TERRY,  
S. W. HARPER.